

May 19, 1964

R. T. CARPENTER

3,133,855

64 R. T. CARPENTER 3,  
MINIMIZING SCRATCHES IN A BLADE COATED PAPER WEB  
BY ROUGHENING THE SMOOTH SIDE OF THE WEB  
PRIOR TO THE BLADE COATING OPERATION  
1961

Filed July 24, 1961

3 Sheets-Sheet 1



May 19, 1964

R. T. CARPENTER

3,133,855

MINIMIZING SCRATCHES IN A BLADE COATED PAPER WEB  
BY ROUGHENING THE SMOOTH SIDE OF THE WEB  
PRIOR TO THE BLADE COATING OPERATION

Filed July 24, 1961

3 Sheets-Sheet 2

*Fig. 2.*



*Fig. 3.*



*Fig. 4.*



May 19, 1964

R. T. CARPENTER

3,133,855

MINIMIZING SCRATCHES IN A BLADE COATED PAPER WEB  
BY ROUGHENING THE SMOOTH SIDE OF THE WEB  
PRIOR TO THE BLADE COATING OPERATION

Filed July 24, 1961

3 Sheets-Sheet 3



1

3,133,855

**MINIMIZING SCRATCHES IN A BLADE COATED PAPER WEB BY ROUGHENING THE SMOOTH SIDE OF THE WEB PRIOR TO THE BLADE COATING OPERATION**

Russell T. Carpenter, Neenah, Wis., assignor to Kimberly-Clark Corporation, Neenah, Wis., a corporation of Delaware

Filed July 24, 1961, Ser. No. 126,047  
5 Claims. (Cl. 162—135)

This invention relates to the production of coated paper and is more specifically directed to a method of formation of the paper web to particularly adapt the web to blade coating operations.

It has been recognized that paper produced in web form either on a Fourdrinier or cylinder machine is subject to a variation between opposite sides of the web termed in the industry "two-sidedness." In essence, this term relates to a web in which the wire side of the web is more rough than the upper or felt side. More in detail, in the formation of the web, that side which is produced in contact with a traveling screen or cylinder and dewatered, and then dried, loses in the course of the operation more of the fiber fines and fillers commonly used in the paper furnish than does the upper or felt side. Thus there is a greater concentration of paper fines and fillers in the upper or felt side of the web or sheet and this latter side therefore exhibits a greater smoothness.

The characteristic of "two-sidedness" tends to carry through the operation even when the paper web is well coated on both sides with the usual mineral coating. Compensating steps therefore are normally undertaken to eliminate the "two-sidedness" characteristic. Commonly, such steps have involved providing the relatively rough wire side in such manner that it more closely approaches the surface characteristics of the smoother upper side.

This present invention is directed to an opposite feature and involves the roughening of the upper or felt side and the presentation of the web with the opposed sides roughened or in roughened condition to a blade coating device.

In blade coating devices the web is usually provided with an excess of the coating material by suitable means such as a roller applicator, a pond or the like; the excess of coating material on the web is then bladed off to effect a smooth coating. The blade commonly employed for such purpose is somewhat flexible. In some instances the coated web passing beneath such blade is subject to receiving fine scratches which affect to some extent the quality of the paper for certain printing operations such as those of letterpress and rotogravure.

Factors which affect the development of these fine scratches appear to include the formation of small particle aggregates in the coating material itself as well as, in some rare instances, foreign particles which may be swept from the fluid lines of the apparatus. In addition, in the usual coating machines employing recirculation systems for the coating material, hardened particles and coated fiber fines may be passed around through the system.

The flexible blade then tends to retain such particles and to promote the production of fine scratch marks.

Roughening of the upper or felt side of the web before presentation of the web to the blade coating device for coating of the upper or felt side apparently permits small particles, whatever their source, to pass through the blade. The particles tend to be immersed in fluid coating material in the irregularities of the web. Accordingly, the particles passed do not interfere with the uniformity of the surface of the coated web, since they are surrounded by fluid coating material in their passage of the blade. In addition, the web itself with respect to two-sidedness is

2

improved. Additionally, by the roughening of the web, compensating steps such as the provision of somewhat different coating compositions for each side of the web may be substantially eliminated. In this connection it is to be noted that the blade coating method itself is desirable due to the tendency of such method to provide both sides of the web with comparable printing characteristics.

Roughening of the web in accordance with the invention is achieved by imposing a continuous controlled pattern on the upper or felt side of the base web. Treatment while the web is well wetted facilitates the roughening action; heavier basis weight webs which customarily tend to scratch somewhat more readily are adapted well for the practice of this invention.

Roughening is effected in the papermaking operation prior to passage of the web to the coating device for the upper or felt side; suitably, the dandy roll, a felt mark, or a steel stack may be provided to impose the pattern. Suitably also, both sides of the web may be impressioned to aid uniformly from one side to the other.

Accordingly, a primary object of the present invention is to provide a new and novel blade coating process in which the web on the papermaking machine is provided with a controlled pattern prior to being passed to the coating device.

Another and important object of the invention is to provide novel apparatus arrangements for the practice of the invention.

These and other allied objects of the invention will be more fully understood by reference to the following detailed description and accompanying drawings wherein:

FIG. 1 diagrammatically illustrates a paper-making machine adapted for carrying out embodiments of the invention.

FIG. 2 is a view in perspective of a dandy roll useful in the practice of the invention.

FIG. 3 is an enlarged fragmentary view illustrating the wire of the dandy roll cover of FIG. 2.

FIG. 4 is a sectional view taken on line 4—4 of FIG. 3.

FIG. 5 is a fragmentary view illustrating the application of a felt in the practice of the invention.

FIG. 6 is an enlarged sectional view taken on line 6—6 of FIG. 5.

FIG. 7 is a fragmentary and elevational view illustrating an embodiment in which cooperating knurled rolls serve to effect roughening in accordance with the invention.

FIG. 8 is an enlarged and fragmentary view illustrating more particularly the cooperation of the rolls of FIG. 7.

Referring to the drawings and initially particularly to FIG. 1, the furnish for the formation of the paper web W is flowed from a head box 1 through a slice 2 over an apron 3 to a traveling Fourdrinier wire 4. Wire 4 is carried on breast roll 5 and couch roll 6. A number of supporting table rolls are designated by the numeral 7 and perform the usual function of supporting the wire and pumping the water from the web, breaking the surface tension of the water contained in the forming web and thereby promoting drainage. The usual stretch rolls are designated at 8, and the guide roll which serves to maintain the wire limited in its lateral oscillation is indicated at 9. As is well known, such Fourdrinier wires oscillate from side to side to provide some cross lay of the fibers in the web. Section boxes are designated at 10 and serve both to support the moving wire and to further aid in withdrawal of water from the web. Couch roll 6 is commonly driven to effect wire rotation.

In the passage of the forming web over the wire, water

is flushed through the wire and fines of mineral material as well as small fibers from the furnish are flushed primarily from the wire side S of the web contacting the wire. This action occurs at both the table rolls and the suction boxes. The formed web as it passes the suction boxes contains usually in excess of 80% of water. Suitably, the couch roll 6 is also a suction roll and so contributes to the withdrawal of water from the traveling web. Under such conditions the web leaving the couch roll will still contain between about 75%-85% of water but is self-supporting.

As illustrated in FIG. 1, a dandy roll 11 is provided in contact with the traveling web on the felt side F. At some distance prior to the couch roll between the dandy roll and the couch roll, and indicated by the numeral 12, is a line which extends transversely of the web and is termed the dry line. The dry line is indicative of a condition of the paper during formation; essentially, the dry line is that position on the forming wire in which the forming web no longer has free water covering the surface of the web but has water primarily only within the interstices of the fibers. Customarily, it is desired to withdraw water from the web uniformly across the width so that the dry line is substantially at right angles with the web.

From the couch roll the traveling web passes to the press section. Included in a press section may be a suction press area designated 18 and its cooperating press felt indicated at 19. A plain press is identified by the numeral 20 and its cooperating press felt by the numeral 21. The numerals 22 and 23 indicate cooperating pressure rolls. This press section as thus described is conventional and the water content of the web leaving the press section is approximately 60-70%.

The drier 25 is comprised of a plurality of drums 26 and the paper web, in its passage, is supported by a bottom drier felt 27 and the top drier felt 28. Conventionally, the moisture content of the web leaving the drier is approximately 4-6%, and the web is in substantial equilibrium with the atmosphere.

As the web leaves the drier and passes in the direction indicated by the arrows, it enters a steel stack 30 composed of a stack of rolls the lower of which is positively driven and the others of which are turned by friction. The web leaving the breaker stack is at a temperature of approximately 130-150° F. and is passed, as indicated in the figure, directly to coating apparatus generally designated by the numeral 35.

This coating apparatus includes a retainer trough 36 for a pond of coating composition 37 in which applicator 38 rotates in the direction indicated by the arrow. Pressed into contact with the applicator 38 is a rubber covered backing roll 39 which travels in an opposite angular direction to that of the applicator roll and forms with the applicator roll a nip 40. The web, traveling at the speed of the backing roll, passes through the nip through a dwell distance 41 to a knife blade 42 supported in pressed contact in any convenient manner by the web and backing roll. As illustrated in FIG. 1, coating material applied at the nip 40 in excess to the felt side is directed to the blade 42 where the excess coating material is removed and recirculated to the coating material system (not shown). From the blade 42 the web passes over drum drier 44, through driers 45 over tensioning roll 46 and around guide roll 47 to the coating device 43 for application of coating material to the wire side S of the web.

The composition which is supplied to the web is conventional and in actual practice may cover a wide range of solids contents and viscosities. Exemplary of the composition is coating material having the following characteristics and components: 100 parts by weight of coating clay, 16 parts by weight of pearl starch (enzyme converted), 1% of soap, caustic to adjust the pH to about 7.2, and water sufficient to provide the solids con-

tent at about 59%. The specific gravity of such a composition is approximately 1.42 and conventionally has a viscosity of about 69.5° Brookfield (measured at 100 r.p.m. with a #6 spindle at 50° C.). In the practice of this invention in the manner now to be described, the same coating composition may be applied to each side of the web.

In the apparatus arrangement described hereinbefore and which, as thus broadly set forth, is conventional, several mechanical changes may be employed to produce the felt or upper side of the web in a roughened condition. Preferably, the web is acted on mechanically while it is still in a somewhat plastic state, although the imposition of the desired roughening pattern may be effected by impressioning of the dried web itself.

More specifically, the dandy roll 11 (FIG. 1) may be provided with a cover having a configuration such as that illustrated in FIGS. 2-4 inclusive. Pressed engagement of the dandy roll with the web on the Fourdrinier wire 20 serves to indent, roughen, and render somewhat open the usually smooth upper felt side. The dandy roll preferably for this purpose is positioned on the wire somewhat forwardly of the dry line so that it contacts the web while the web is thoroughly wetted. The dandy roll itself, as illustrated in FIGS. 2-4 inclusive, is provided with a wire 50 formed of a series of parallel warp wires 51 and a series of parallel shute wires 52. As shown, wire 50 has a twill weave in which each of the warp wires 51 passes over its shute wires 52 and under a third shute wire to provide relatively high and long warp knuckles 53. The shute wires themselves each have relatively low knuckles beneath which the warp wire passes. The terms warp and shute are here used in the conventional sense in connection with wire cloth weaving wherein the warped wires extend longitudinally of the loom and are crimped to a greater extent than the shute wires.

The wire illustrated in FIGS. 3 and 4 may be utilized with either side forming the outer web contact surface of the dandy roll. Further, other weaves which provide a rough surface may be employed. In many instances the Fourdrinier wire itself will have a rough surface, and the dandy roll surface may correspond to it.

Close correspondence between the sides of the forming web, of course, minimizes two-sidedness in the web as well as aiding the subsequent blading operation.

In FIGS. 5 and 6 a felt arrangement 55 adapted to have felt 56 contact the upper side of the moving web W is illustrated. Felt 56 is marked or provided with alternate raised and lowered portions 57 and 58 respectively. These markings may be in any desired pattern to provide a roughened surface of the web. The felt 56 thus provides an alternative method of imposing a surface configuration on the web which, at the press section, is still relatively plastic and impressionable by the moving felt.

FIGS. 7 and 8 illustrate a pair of cooperating rolls 22a, 23a which have been substituted for the smooth rolls 22, 23. Roll 22a has a surface 60 knurled as indicated at 61 to cooperate with the surface 62 which is also knurled as indicated at 63. In this instance both web surfaces are altered to achieve close correspondence between the opposite sides of the web.

In a manner similar to that described in connection with FIGS. 5 and 6 the top drier felt 28 (FIG. 1) may be marked to impose a controlled pattern on the web as it passes over the drier. Similarly, the lower stack rolls in stack 30 may be knurled, relieved, formed with protuberances or recesses, or otherwise provided with a pattern for marking and roughening the web W as it moves through the stack. In general, the roughening action tends to affect the sheet less when the pattern is imposed while the sheet is plastic.

Thus, in effect, to achieve improved blade coated paper webs it is only necessary to provide the felt side roughened prior to passing the web to the coating device and

then to blade coat the so roughened web. In general, the procedure of invention, while applicable to all webs, is more important in connection with heavier basis weight webs. It is in this area particularly that scratching of the coated sheet may occur.

It will be understood that this invention is susceptible to modification in order to adapt to different usages and conditions and, accordingly, it is desired to comprehend such modifications within the invention as may fall within the scope of the appended claims.

What is claimed is:

1. In a process for producing printing paper in which a newly formed traveling web of paper having a relatively smooth and a relatively rough side is dried, coated, and subjected to a knife blade operation while supported on a backing roll to smooth and remove excess coating from the web, the steps of imposing a configurated pattern on the smooth web side prior to the coating thereof to roughen the said side, subsequently applying an excess of aqueous mineral coating containing pigment and adhesive to the said side, and thereafter blading the excess of coating from said side and smoothing the remaining coating thereon.

2. In a process for producing printing paper in which a newly formed traveling web of paper having a relatively smooth and a relatively rough side is dried, coated, and subjected to a knife blade operation while supported on a backing roll to smooth and remove excess coating from the web, the steps of imposing a configurated pattern on the smooth web side while the web is wet and somewhat plastic and prior to the coating of said side to roughen the said smooth side, subsequently applying an excess of aqueous mineral coating containing pigment and adhesive to the said side, and thereafter blading the excess of coating from said side and smoothing the remaining coating thereon.

3. In a process for producing printing paper in which a newly formed traveling web of paper having a relatively smooth and a relatively rough side is dried, coated, and subjected to a knife blade operation while supported on a backing roll to smooth and remove excess coating from the web, the steps of imposing a configurated pattern on the smooth web side while the web is wet and somewhat plastic and before the forming web reaches the dry line and prior to the coating of said side to roughen the said smooth side, subsequently applying an excess of aqueous mineral coating containing pigment and adhesives to the said side, and thereafter blading the excess of coating from said side and smoothing the remaining coating thereon.

4. In a process for producing printing paper in which a newly formed traveling web of paper having a relatively smooth and a relatively rough side is dried, coated, and subjected to a knife blade operation while supported on

a backing roll to smooth and remove excess coating from the web, the steps of imposing a configurated pattern on the smooth web side while the web is wet and somewhat plastic and prior to the coating of said side to roughen the said smooth side, to the same extent as the mentioned rough side subsequently applying an excess of aqueous mineral coating containing pigment and adhesive to the said side, thereafter blading the excess of coating from said side and smoothing the coating thereon, and subsequently coating the second and opposite side of the paper web with the same coating composition.

5. The process of producing printing paper which comprises:

- (a) forming a traveling paper web having a relatively smooth felt side and a relatively rough wire side;
- (b) while the web is formed and wet and plastic imposing a continuous controlled pattern on the felt side of the web to roughen and open the felt side;
- (c) drying the web with the felt side in the roughened open condition;
- (d) applying to the roughened open and dried felt side an excess of an aqueous mineral coating composition containing pigment and adhesive;
- (e) carrying the web with the excess of coating composition thereon on a rubber covered backing roll to a flexible blade pressed against the web on the backing roll;
- (f) removing the excess of aqueous mineral coating composition from the traveling web with the flexible blade while smoothing the remainder of the coating on the web;
- (g) said roughened open condition of the web providing for passage of small particle aggregates in the coating remaining on the web without substantial scratching of the coating; and
- (h) subsequently drying the coated web.

#### References Cited in the file of this patent

#### UNITED STATES PATENTS

|           |                 |       |               |
|-----------|-----------------|-------|---------------|
| 1,369,186 | Perry           | ----- | Feb. 22, 1921 |
| 1,501,493 | Koplin          | ----- | July 15, 1924 |
| 2,156,046 | Alt             | ----- | Apr. 25, 1939 |
| 2,186,957 | Collings et al. | ----- | Jan. 16, 1940 |
| 2,216,803 | Benda           | ----- | Oct. 8, 1940  |
| 2,287,161 | Ball            | ----- | June 23, 1942 |

#### OTHER REFERENCES

Calkin: "Modern Pulp and Papermaking," 3rd edition, Reinhold Publishing Corp., N.Y., 1957, page 331. (Copy in Scientific Library.)

McGraw-Hill, "Manufacture of Pulp and Paper," vol. 5, McGraw-Hill Book Co., N.Y., 1939, section 6, page 55 31. (Copy in Div. 25.)